

Patented Mar. 24, 1925.

1,531,140

# UNITED STATES PATENT OFFICE.

GEORGE SCHNEIDER, OF LA VALE, MARYLAND, ASSIGNOR TO THE AMERICAN CELLULOSE & CHEMICAL MANUFACTURING COMPANY, LTD., OF NEW YORK, N. Y.

## METHOD OF FORMING ELECTRODEPOSITS.

No Drawing.

Application filed January 19, 1924. Serial No. 687,387.

To all whom it may concern:

Be it known that I, GEORGE SCHNEIDER, a citizen of the United States, residing at La Vale, Cumberland, State of Maryland, have 5 invented certain new and useful Improvements in Methods of Forming Electrodeposits, of which the following is a specification.

This invention relates to a method of 10 electrodepositing a metal upon a prepared object in such manner that it can be easily removed therefrom. The deposit may be of nickel, copper, or other suitable metal or combination of metals, and the object on 15 which the deposit is formed may be of similar material.

When metal is plated electrolytically directly upon an object made of the same or another metal or metals, it is usually very 20 difficult to separate or strip the plated metal from the object plated. This is particularly the case if an electrodeposit of nickel is made upon a copper object constituting the cathode.

25 The object of my invention is to enable a metal particularly nickel or copper electroplated upon a metal object particularly copper or nickel to be stripped or removed therefrom with great facility or in other 30 words, to so conduct the process as to prevent the deposited metal from strongly adhering to the object plated.

In carrying out my invention the object to be plated is prepared by first forming 35 upon the surface thereof an extremely thin electrodeposit which serves as an intermediate layer or lamination. Such thin deposit should have tenacious properties sufficient to allow the final deposit of plate 40 metal to adhere firmly to the object being plated during the plating operation in order to obtain the maximum definition of detail effect on the deposit, and also such non-adhering properties as to allow the final deposit to be easily removed or stripped without injuring the surface of the deposit or of 45 the object plated, and thirdly in some cases this thin intermediate layer should be of such character that it will not interfere 50 with the transference of the high polish from the surface of the object plated to the deposit or duplicate.

Many materials for such an intermediate layer are not suitable for the purposes above 55 mentioned, being either non-adherent or ad-

herent to a greater extent than required. Arsenic, electrically deposited, from an appropriate solution is only partially successful for the purposes mentioned because it does not permit the plate metal to adhere 60 sufficiently to the object plated to obtain a deposit of the desired thickness, inasmuch as it is under electrical tension while being formed and would separate from the object before completion.

65 I have discovered that if this very thin deposit or intermediate layer be formed of an admixture of nickel, copper or other suitable metal or metals and arsenic in the proper proportions, the desired results are 70 satisfactorily obtained. By employing for this layer the substances just mentioned, the desired final deposit can be made of the required thickness for use and it will adhere 75 firmly to the object treated while being deposited and when the deposition is completed the final deposit can be easily stripped from said plated object.

When nickel and arsenic are used the desired proportions of these may be defined or 80 ascertained by the color of the deposit, which latter is extremely thin, being only a fraction of a thousandth of an inch in thickness and the color appears as a mere blush or flash upon the polished surface of the 85 object and should, I have found, be of a steel blue tint.

While arsenic deposits as dead grayish black and nickel as bright white, the two 90 when combined in proportions, as above described, produce a deposit of the steel blue color above mentioned and the polish of the treated object is retained.

The treated object after being flashed with 95 the materials above mentioned may be plated in a suitable electroplating bath of copper, nickel, or other desired metal and a deposit of the desired thickness of metal is thus obtained. When the last named deposit has reached the desired thickness, the plated object may be withdrawn from the bath and the electroplated deposit may be readily stripped or removed. The intermediate thin layer is more or less absorbed by the 100 final deposit and in no way detracts from the exact duplication produced in the stripped deposit of any of the detail effect 105 present on the surface of the object plated.

In this way metals of many kinds may be 110 deposited singly or in combination as a

laminated sheet or as a mixed deposit and readily stripped from an object made of the same or other metal or metals.

In some cases instead of forming the intermediate layer of nickel and arsenic, other suitable metal may be used in place of nickel, but in all cases I prefer to use arsenic in connection with the metal.

I have stated that the proper proportions 10 of nickel and arsenic maybe ascertained by the color of the film or intermediate layer produced, this color being of a steel blue tint. When another metal is used in place of nickel, the color of the film may be different but in all cases the proportion of arsenic to metal is three to four parts arsenic to one of the metal used.

When practicing the process for the making of nickel deposits I preferably proceed 20 as follows though the scope of my process is in no way confined to this particular example. The object to be treated is used as a cathode and may be of copper or other suitable metal or metals. It is first polished 25 and either with or without a nickel face is placed in a bath consisting of an admixture of the usual nickel plating salts and white arsenic and/or sodium or potassium arsenite in the correct proportions. For example a 30 plating bath suitable for the purpose would consist of:

13 parts nickel ammonium sulphate,  
4 parts zinc sulphate,  
4 parts sodium chloride,  
35 5 parts ammonium carbonate,  
8 parts sodium cyanide,  
1 part sodium bisulphite,  
20 parts arsenite (9 1/3 parts  $As_2O_3$ , 10 2/3 parts NaOH).

40 The plating operation is conducted for a very brief period and at a low current density and tension. A plating period of two minutes at a temperature of 30° C. and a current density of 1/3 to 1/2 ampere 45 per sq. decimeter at four to five volts has been found to give the desired "flash." The cathode is then washed and without drying is placed in a nickel plating bath and treated in the usual manner well known 50 in the art until the desired thickness of deposit is obtained. As soon as such thickness is obtained, the plated object is removed from the bath and the deposit is stripped or removed from the object and is 55 ready for use. The cathode or object may be again prepared and plated in the manner before described.

My invention may be used in the manufacture of various articles, such as talking 60 machine records, printing plates, etc. When making talking machine records, the member, known in the art as the "mother," is according to my invention treated in the manner before described to produce by electrodeposition on its surface a thin layer

i. e. a flash or film of arsenic and nickel. This deposited material serves as an intermediate non-adherent or anti-adherent film and on this film I deposit a sufficient amount of nickel to produce the desired nickel shell 70 to be used in the manufacture of records. For economic reasons this shell is often given a subsequent treatment in a copper plating bath until of the desired thickness. The character of the intermediate layer or film, which is of very minute thickness, 75 must be such that the subsequent depositing of the pure nickel thereon can be carried to completion without separating or stripping under electrical tension from the mother member on which it is deposited. The film should also have such non-adherent properties as to enable the final deposit of nickel to be readily separated when completed. One of the features of my invention, therefore, is its adaptability to the manufacture of talking machine records 80 from shells made of nickel which are capable of producing records of superior quality over those made from copper or nickel faced copper shells and, furthermore, it will be observed that in the manufacture of such nickel shells I am able to strip the nickel shells from the mother or foundation on which they are formed with great facility 85 without in any way injuring either the record forming surface or the surface of the "mother."

I claim as my invention:

1. The method hereinbefore described of 100 forming a metal deposit upon an object to be plated, which consists in first forming on the surface of the object an intermediate deposit of a mixture of arsenic and one of the heavy metals, and then depositing a plating metal on such treated object until a plating of the desired thickness is obtained.

2. The method hereinbefore described of 105 forming a metal deposit upon an object to be plated, which consists in first forming on the surface of the object a deposit of a mixture of one part nickel and three to four parts arsenic and then depositing a plating metal on the treated object until a plating of the desired thickness is obtained.

3. The method hereinbefore described of 110 forming metallic negatives of an object, which consists in first "flashing" or thinly plating the object with a mixture of arsenic and one of the heavy metals and then depositing a plating metal on this treated object until a plating of the desired thickness is obtained which may be removed.

4. The method hereinbefore described of 115 forming a negative of an object in electro-deposited nickel, which consists in first treating the surface of the object with a mixture of one part nickel and three to four parts arsenic and then electrodepositing nickel 120 on such treated object until a plating of the 125

desired thickness is obtained, which may be removed.

5. The hereinbefore described method of forming a metallic shell for the manufacture of talking machine records, which consists in forming on a metal surfaced member or "mother" a thin film or "flash" of an electrodeposited mixture of arsenic and one of the heavy metals, and then electrodepositing a 10 plating metal on said treated member or "mother" until a shell of the desired thickness is obtained which may be removed.
6. The hereinbefore described method of forming a nickel shell for the manufacture 15 of talking machine records, which consists in forming on a metal surfaced member or "mother" a thin film or "flash" of electrodeposited nickel and arsenic, and then electrodepositing nickel on said treated member until a nickel shell of the desired thickness is obtained which may be removed.
7. The hereinbefore described method of forming metallic shells for the manufacture 20

of talking machine records, which consists in forming on a metal surfaced member a 25 thin film or flash of an electro deposited mixture of arsenic and one of the heavy metals, then electrodepositing a plating metal on said treated member until a shell of the desired thickness is obtained and then 30 stripping or removing the shell from said member.

8. The hereinbefore described method of forming a nickel shell for the manufacture 35 of talking machine records, which consists in forming on a metal surfaced member or "mother" a thin film or flash of electrode- deposited nickel and arsenic, then electrode- 40 positing nickel on said treated member until a shell of the desired thickness is obtained and then stripping or removing the nickel shell from said member.

In testimony whereof, I have hereunto subscribed my name.

GEORGE SCHNEIDER.